

## UNITED STATES PATENT OFFICE

2,130,460

## TREATING CELLULOSIC FIBER

John Gwynant Evans, Blackley, and Sidney Arthur Slater, Stretford, England, assignors to Imperial Chemical Industries Limited, a corporation of Great Britain

No Drawing. Application March 23, 1936, Serial No. 70,548. In Great Britain March 25, 1935

4 Claims. (Cl. 19—66)

It is known that certain difficulties are encountered in the spinning of staple fiber, that is fiber composed of short lengths of viscose, acetate and similar rayon, into yarn owing to the tendency of the fibers to slip when being twisted. Similar, though less pronounced difficulties are met with in the spinning of the smoother cellulosic fibers such as flax and ramie or in the spinning of short staple cotton fiber such as some kinds of Indian cotton, which in order to obtain a commercially useful thread, have to be spun with a considerable amount of twist.

It is an object of the present invention to avoid or minimize these difficulties. It is a further object to produce spun thread of improved properties. It is a further object to produce new and useful compositions of matter. Other objects will become apparent as the description proceeds.

We carry out our invention by treating cellulosic fiber of whatever origin, whether natural or artificial or composed of pure cellulose or of cellulose derivatives, with a solution or emulsion of colophony.

It is known to treat rayon fabric, i. e. already woven material, with resin acids or alkali metal salts of resin acids to produce on the surface of the component threads a deposit which imparts to it a non-displacement finish (see British specification 388,157) but it was not to have been expected from anything disclosed in that specification that treatment of fiber according to the present invention would facilitate its spinning as above mentioned or indeed that such treatment would not impede spinning or make it impossible.

Our preferred method of applying the colophony is from an aqueous solution or emulsion dissolved or emulsified by means of alkali in conjunction with other assistants used in textile treatments, more especially softening agents, antiseptics, stiffening agents, weighting agents. The fiber is immersed in a suitable solution until permeated, excess solution removed and the fiber dried. There is thus obtained a new composition of matter, namely unspun cellulosic fiber attached to colophony and any assistant which may have been employed in conjunction with colophony. This improved composition possesses improved properties, whether in the unspun or spun condition, as compared with ordinary fiber, as has been described.

The following example illustrates but does not limit the invention. The parts are by weight.

## Example

Staple viscose fiber is treated for 16 minutes at 45° C. in 1000 parts of water containing 10 parts of a mixture or emulsion consisting of—

|                       | Parts |
|-----------------------|-------|
| Glue                  | 250   |
| Cetyl sodium sulphate | 75    |
| Colophony             | 330   |
| Caustic soda flakes   | 35    |
| Salicylic acid        | 7½    |
| Water                 | 1,425 |
|                       | 15    |

After treatment the material is centrifuged and dried. The fiber is then spun in the normal manner and owing to the increased adherence between the fibers, a yarn of increased strength with a given twist results. Short staple cotton fiber, flax and ramie fiber may be similarly treated in order to improve their spinning qualities.

We claim:

1. The process which comprises treating smooth, staple cellulosic fibers with a solution containing a small amount of colophony, cetyl sodium sulphate, and caustic soda.

2. Staple cellulosic fibers produced by the process of claim 1.

3. The process which comprises treating smooth staple filaments of a chemically modified cellulose taken from the class consisting of viscose and cellulose acetate with a solution obtained by mixing

|                       | Parts |
|-----------------------|-------|
| Glue                  | 250   |
| Cetyl sodium sulphate | 75    |
| Colophony             | 330   |
| Caustic soda          | 35    |
| Salicylic acid        | 7.5   |
| Water                 | 1,425 |

and adding 10 parts of the mixture to 1000 parts of water.

4. Staple fibers obtained by the process of claim 3.

JOHN GWYNANT EVANS.  
SIDNEY ARTHUR SLATER. 50